# EUROPEAN PATENT APPLICATION

(11) **EP 0 749 805 A1**
(43) Date of publication of application: **27.12.1996**
(21) Application number: 95610037.4
(22) Date of filing: 20.06.1995
(51) Int. Cl.: B24B 1/04

(54) **A diamond polishing method and apparatus**

(71) Applicant: Snitka, Valentinas, Kaunas 3000 (LT)
(72) Inventor: Snitka, Valentinas, Kaunas 3000 (LT)
(74) Representative: Plougmann, Vingtoft & Partners A/S

(57) **Abstract**

A method and an apparatus for polishing a diamond surface by utilization of ultrasonic vibrations are provided whereby surface roughness of a diamond surface can be reduced to a level suitable for e.g. mechanical, optical, and semi-conductor applications in a very short time period. The polishing apparatus comprises a frame (7) means (10) for mounting a diamond polishing member on said frame, means (11) for mounting a diamond member on the frame, means for moving a polishing surface defined on the polishing member into contact with a surface of the diamond member to be polished, and ultrasonic transducer means for moving the diamond and polishing surfaces in relation to each other so as to polish the diamond surface. Typically, the diamond surface to be polished is the surface film, e.g. of a synthetically produced diamond film, e.g. of a CVD-diamond film. The short polishing time period needed is thought to be due to one or more effects of ultrasonic vibration such as fracture of asperities, diffusion of carbon of diamond, oxidation of carbon of diamond, etc.

## Description

### FIELD OF THE INVENTION

The present invention relates to a method and an apparatus for polishing a diamond surface by utilization of ultrasonic vibrations of a polishing surface relative to the diamond surface to be polished.

### BACKGROUND OF THE INVENTION

Diamond, such as diamond film, has received considerable attention in recent years because of its unique combination of optical, thermal, mechanical, chemical and semiconductor properties.

Diamond has excellent transmitting properties of electro-magnetic radiation over a wide wavelength range extending from the ultraviolet region to the far infrared and over much of the microwave radar frequencies.

The thermal conductivity of diamond is the highest among all known materials. At room temperature it is a factor of five greater than copper and over an order of magnitude more effective than commonly used thermally conductive insulators such as aluminium nitride or beryllium oxide.

Also, diamond is an excellent electrical insulator due to its large band-gap and purity and this combination of high insulation and high thermal conductivity makes diamond an ideal material for heat sinks for power electronic components and semiconductor lasers and for packaging of electronic and optoelectronic devices.

Diamond is the hardest known material and has one of the lowest coefficients of friction making it an ideal material for cutting tools and wear resistant components.

Further, diamond is highly resistant towards chemicals due to its chemical inertness, making it an ideal material for protection of components in corrosive environments.

The full industrial exploitation of this unique combination of properties has been limited by the scarcity and limited size of high-purity natural or synthesised diamond.

However, recently new methods of artificially synthesizing diamond have been developed, which are expected to provide synthesized diamond at reduced cost so that the application of diamond for the various purposes mentioned above is getting more and more economical.

Presently the most promising production method of synthetic diamond is the chemical vapour deposition method. This method provides a very pure synthetic polycrystalline diamond by dissociation of mixtures of carbon-based gases and hydrogen below atmospheric pressure and deposition of a layer of high-purity, polycrystalline diamond on a heated substrate. Diamond films of large area of coverage and large thickness may now be produced either on substrates or as self-sustained diamond wafers.

A major obstacle to the wide spread use of diamond films in the above-mentioned applications is the surface roughness. Growth of the diamond phase on a non-diamond substrate is initiated by nucleation either at randomly seeded sites or at thermally favoured sites due to statistical thermal fluctuation at the substrate surface. Based on growth temperature and pressure conditions, favoured crystal orientations dominate the competitive growth process. As a result, the grown films are polycrystalline in nature with relatively large grain size (> 1µm), and terminating in very rough surfaces with roughnesses ranging from about few tenth of a micron to tens of microns.

Further, the film surface formed at the beginning of the diamond nucleation and initial growth may have undesirable properties because of small grain size with many grain boundaries with a high risk of impurity segregation therein.

Therefore, it is necessary to polish the diamond film surface at the top, and for some applications both at the top and at the bottom of the diamond film to reduce the surface roughness.

As diamond is extremely hard it has, until now, been extremely costly and time consuming to polish diamond surfaces. Traditional mechanical polishing methods using hard abrasive particles or thermochemical, chemomechanical or plasma/laser polishing methods are inadequate because of extremely low polishing rates.

For example, from S. Jin, J.E. Graebner, and T. H. Tiefel: "Thinning and polishing of diamond films by diffusional reaction with metals", SPIE Vol. 1759 Diamond Optics V, 1992, it is known to thin and polish CVD diamond films by diffusional transfer of carbon atoms from the diamond film to a metal (Fe or Mn) of a high solubility of carbon. The diffusion takes place in a furnace chamber heated to 900 °C for 16-48 hours in a flowing argon gas atmosphere. The diffusion process is followed by mechanical polishing on a diamond bonded wheel or by etching in a 50% Hcl solution. Surface roughness below 1µm and thickness reduction of 100 µm in 48 hours are reported.

### SUMMARY OF THE INVENTION

It is an object of the present invention to provide a method of polishing diamond to a surface roughness suitable for mechanical applications.

It is a further object of the present invention to provide a method of polishing diamond to a surface roughness suitable for optical applications.

It is another object of the present invention to provide a method of polishing diamond to a surface roughness suitable for semiconductor applications.

It is still another object of the present invention to provide a method of polishing diamond to a surface roughness suitable for the above-mentioned applications in a short period of time.

It is yet another object of the present invention to provide a method of polishing diamond utilizing diffusion of carbon atoms of the diamond into another material without the need of increasing the ambient temperature of the diamond sample to be polished, e.g. in a furnace.

It is a further object of the present invention to provide a method of polishing diamond utilizing oxidation of carbon atoms of the diamond without the need of increasing the ambient temperature of the diamond sample to be polished, e.g. in a furnace.

According to the invention, the above-mentioned objects are fulfilled by providing a method of polishing a surface of a diamond member by means of a polishing member defining a polishing surface thereon, said method comprising moving the diamond surface into contact with the polishing surface and moving the diamond member relative to the polishing member by ultrasonic transducer means so as to polish the diamond surface by moving the diamond and polishing surfaces in relation to each other.

Further, the above-mentioned objects are fulfilled by providing a polishing apparatus according to the invention, for polishing a surface of a diamond member, said apparatus comprising a frame, means for mounting a diamond polishing member on said frame, means for mounting a diamond member on the frame, means for moving a polishing surface defined on the polishing member into contact with a surface of the diamond member to be polished, and ultrasonic transducer means for moving the diamond and polishing surfaces in relation to each other so as to polish the diamond surface.

Typically, the diamond film surface to be polished is a diamond film surface, typically, produced synthetically.

The term polishing denotes any process of reducing thickness or surface roughness of a component, such as by polishing, planarizing, flattening, thinning, abrading, grinding, etc.

Ultrasonic transducer means may comprise any transducer for generation of ultrasonic vibrations, such as piezoelectric crystals or ceramics, magnetostrictive components, etc.

The polishing surface may be the surface of any material suitable for polishing a diamond surface, materials such as, diamond films, ceramics, such as Al₂O₃, etc., crystals, such as BN, etc., metals, such as Fe, Mn, etc., etc.

Preferably, during initial polishing, the polishing surface is the surface of another diamond film to be polished so that two surfaces of diamond films are polished simultaneously.

It is an important aspect of the present invention that the fragility of diamond material is exploited to increase the mechanical polishing rate of diamond by orders of magnitude. Due to the extreme hardness of diamond, polishing of an asperity of the surface is extremely time consuming. However, according to the present invention, the asperities are broken off as a result of controlled hammering of the two surfaces with asperities against each other. The forces created by the impact of asperities against asperities cause the asperities to break off the surfaces and, further, interlocked asperities fracture as a result of ultrasonic shear forces in the surfaces. As a result, the surface roughness goes down very quickly during this process. Experiments have been carried out wherein the diamond surface roughness has been reduced from an average roughness of approximately 5 µm to approximately 0.2 µm in less than two minutes. The roughness measurements were made by Atomic Force Microscope Nanoscope II and were measured peak-to-peak values (R^{max}) and average toughness (R^{a}).

It is a further important aspect of the present invention that the ultrasonic vibrations create a considerable temperature rise at the interface between the two surfaces vibrating in relation to each other. Temperatures in the range from 700 - 1000 °C may easily be obtained at which temperatures carbon atoms of the diamond may diffuse into the polishing material and/or carbon atoms may transform into graphite and/or carbon may oxidize and/or carbon may react with chemicals to which diamond is inert at lower temperatures, such as at room temperature.

Ultrasonic vibration of the diamond surface to be polished in relation to the polishing surface may comprise velocity components in all three spatial dimensions. However, two-dimensional or one-dimensional vibration may also be utilized. Preferably, for two-dimensional vibrations, the plane defined by the velocity components of the movement is substantially vertical to the diamond surface and, preferably, for one-dimensional vibrations, the velocity component of the movement is substantially tangential to the diamond surface.

During the final phase of polishing, temperatures in the range up to few hundred degrees can be obtained at which temperature the rate of fine polishing is increased.

Further, the rate of polishing may be increased by utilization of one or more liquid(s) containing oxygen, such as water, acids, etc., the liquid being supplied between the polishing surfaces during polishing. The ultrasound vibrations cause cavitations to be induced in the liquid(s) and the temperature in the cavitation bubbles may increase to up to thousands of degrees Celsius and the pressure in the cavitation bubbles may increase to up to tenths of atmospheres producing a high rate of diamond graphitisation and oxidation.

Further, the ultrasonic vibrations may be in the form of standing or travelling waves and the ultrasonic transducer means may operate in any vibrational mode, such as a longitudinal mode, a transversal mode, a torsional mode, etc. and any combination hereof.

To bring a large area of the diamond surface to be polished into contact with the polishing surface and/or to increase the polished surface uniformity, the diamond surface to be polished and the polishing surface may be moved relative to each other by mechanical displacement means so that the two surfaces may rotate relative to each other and/or may traverse relative to each other.

According to the present invention, methods of polishing diamond are provided that utilize one or more of the effects of ultrasonic vibration mentioned above, such as fracture of asperities, diffusion of carbon of diamond, oxidation of carbon of diamond, diamond reacting with chemicals, etc. It is a major advantage of the present method that these effects become active without heating of the environment of the diamond sample, e.g. in a furnace.

According to a preferred a preferred embodiment of the invention, a method is provided comprising the steps of: producing impact interactions between the polishing surface and the diamond surface to be polished by ultrasonic movement of the diamond surface relative to the polishing surface so that surface protrusions of the diamond surface are broken off the diamond surface, and polishing of the diamond surface with a hard material containing oxygen.

According to another embodiment of the invention, a method is provided further comprising the step of: polishing the diamond surface with a material in which carbon is soluble.

Further, one or more active chemicals may be added between the diamond surface to be polished and the polishing surface to increase the rate of polishing and/or to decrease the resulting surface roughness of the diamond surface. Typically, the chemicals are oxidants, such as peroxides, etc. Preferably, a fused oxidizer, such as KNO₃, etc, is used due to its strong reactive etching affinity towards diamond. The polishing rate can be increased by ultrasound induced cavitation.

### BRIEF DESCRIPTION OF THE DRAWINGS

The invention will now be described by way of example and with reference to the accompanying drawings in which:
Fig. 1 is a scanning electron microscope (SEM) image of the morphology of the growth surface of a typical as-deposited diamond sample,
Fig. 2 is an atomic force microscopy (AFM) image of the morphology of the growth surface of a typical as-deposited diamond sample,
Figs. 3, 4 and 5 show the SEM images of diamond-by-diamond polished samples,
Fig. 4 shows large presence of wear debris around the polished grains,
Fig. 5 shows the polished diamond surface cleaned from wear fragments,
Figs. 6 and 7 show the AFM 3D image of the diamond polished by alumina ceramics,
Figs. 8, 9 and 10 show lateral cross-sections of the unpolished film, the partially polished film and the fully polished film,
Figs. 11, 12 and 13 show the Raman shift spectra of the as-deposited film, after 10s polishing and after 60s polishing,
Fig. 14 shows a XPS spectrum of the alumina ceramic polished diamond,
Fig. 15 shows the friction coefficient versus polishing time,
Fig. 16 shows an AFM image of a typical polished crystallite,
Fig. 18 shows a polishing apparatus,
Fig. 19 shows the velocity components u₁ and u₂ of the elliptical motion at the interface between the diamond surface and the polishing surface, and
Fig. 20 shows another polishing apparatus.

### DETAILED DESCRIPTION OF THE DRAWINGS

The polishing apparatus shown in Fig. 18 comprises an ultrasonic motor, wherein an elliptic movement as indicated in Fig. 19 is created at the interface between a steel slider 1 and a piezoelectric stator 2. The steel slider 1 is pressed onto the stator surface and is put into motion by frictional forces at the interface in that the tangential component of the frictional forces acts as a driving force and the normal component of the frictional forces controls the magnitude of the frictional forces. Speed and direction of motion can be modified by changing the phase shift between the components u₁ and U₂ shown in Fig. 19. The elliptical motion at the interface is produced by sinusoidal vibrations of the two longitudinal vibrators 3, 4 positioned substantially orthogonally to each other.

Fig. 20 shows an alternative embodiment of the invention with two piezoceramic blocks 5, 6, the piezoceramic block 5 working in the longitudinal vibration mode and the piezoceramic block 6 working in the torsional vibration mode, a housing 7, a bolt 8, an insulator 9 between the two piezoceramic blocks 5, 6, two diamond sample holder 10, 11, two diamond samples 12, 13, a bearing 14, a spring 15 to press the two diamond samples 12, 13 against each other, and a shaft 16.

Polishing were performed with the apparatus shown in Fig. 18 with a excitation frequency of 20 kHz, a contact load of 20 N, a slider movement speed of 40 mm/s and a environment relative humidity of app. 65%.

Friction and wear tests were carried out using a pin-on-plate type tribometer constructed with the same design of the polishing apparatus.

Figs. 1 and 2 show the morphology of the growth surface of a typical as-deposited diamond sample. Fig. 1 is a scanning electron microscope (SEM) image and Fig. 2 is an atomic force microscopy (AFM) three-dimensional (3D) image made with constant height mode, respectively. It is seen that the AFM does not introduce artifacts in the surface image and, therefore, the AFM profile is accurate to measure the roughness of the samples.

Figs. 3, 4 and 5 show the SEM images of diamond-by-diamond polished samples. Fig. 4 shows large presence of wear debris around the polished grains. Fig. 5 shows the polished diamond surface cleaned from wear fragments. The Rₘₐₓ roughness has decreased from about 3 µm to about 0.5 µm.

Figs. 6 and 7 show the AFM 3D image of the diamond polished by alumina ceramics which consisted of Al₂O₃ crystallites (95.1%) and SiO₂, BaO, CrO₂, MnO and other oxides.

Figs. 8 and 9 show the correspondent sequence of lateral cross-section from the unpolished film to the final polishing, where the film roughness decreased down to Rₐ of 20 nm.

Figs. 11, 12 and 13 show the Raman shift spectra (a) of the as-deposited film, (b) after 10s polishing and (c) after 60s polishing. The sharp peak at 1330 cm⁻¹ shows that the polishing does not induce the graphitization of the surface, but a higher background in the Raman spectra is clear. this background can be a result from induced defects, wear debris, or a result of tribochemical reactions.

Fig. 14 shows a XPS spectrum of the alumina ceramic polished diamond, where an abundance of ceramic atomic elements can be seen. This suggests that the ultrasonic wear of alumina at diamonds involves probably a tribochemical oxidation of diamonds with the air environment to produce COₓ.

The friction coefficient versus polishing time is presented in fig. 15. The vibration polishing force Fₐ used was 360 kgms⁻² at a frequency of 20 Khz induced by a vibrating mass of 0.05 kg oscillating with an amplitude of 0.5 µm. It is noted that the coefficient of friction of unpolished diamond film is very high when compared to natural diamond and it decreased very fast during polishing. The decrease of friction coefficient versus polishing time suggest that the coefficient of friction depends on the film roughness.

The measured static coefficient of friction between unpolished diamond and steel was 0.5 which is close to the value of the static coefficient of friction measured between alumina ceramic and steel which was 0.65. After polishing, the static coefficient of friction between diamond and steel decreased to 0.2, which was the same value measured for the dynamic friction coefficient of unpolished diamond and steel.

These observations seem to indicate that the high static friction coefficient is related to the indentation of diamond crystallites to the steel.

The correlation of roughness and static friction coefficient is also shown in Fig. 15. It can be seen that the coefficient of friction decreased from 0.55 to 0.1 as the average Rₐ roughness measured by AFM topography was reduced from 270 nm to 11 nm. At the first stage of ultrasonic polishing, the ratchet mechanism plays the main role in the friction between two rough diamond surfaces. The interlocked asperities fracture each other by the presence of ultrasonic shear force and, hence, the surface roughness goes down. However, with rough diamond film sliding against a ceramic material, softer than diamond, material ploughing is expected to play an important role to in the effect of roughness on the friction. It is believed that the temperature at microcontacts in a tribological application may be sufficient to the graphitization of diamond and that this mechanism may be effective in the ultrasonic polishing of diamond by ceramics. Also, the relatively high polishing rate in the ultrasonic polishing suggests that lateral fracture of the diamond grains is probably a concurrent polishing mechanism, specially when roughness is high. In smooth surfaces, tribochemical reactions became important, as well. In this case, ultrasonic excited mechanical vibrations lead to viscoplastic deformation of asperities. The main effect is the damping of vibrations at the frictional interface. It should be pointed out that viscoplastic deformation of asperities is very complex in nature, and therefore it is difficult to model accurately in the macroscopic constitutive law. It is also important to remark that the damping effect is strong at high frequencies, where polishing is more effective, since high frequencies of vibrations are accompanied by high velocities of surface motion.

Fig. 16 shows an AFM image of a typical polished crystallite, where surface plastic deformation can be seen. The correspondent height roughness histogram is presented in Fig. 17. Surface average roughness Rₐ reached was 11 nm in this sample.

## Claims

1. A method of polishing a surface of a diamond member by means of a polishing member defining a polishing surface thereon, said method comprising moving the diamond surface into contact with the polishing surface and moving the diamond member relative to the polishing member by ultrasonic transducer means so as to polish the diamond surface by moving the diamond and polishing surfaces in relation to each other.

2. A method according to claim 1, wherein the diamond member is a diamond film.

3. A method according to claim 1 or 2, wherein the diamond member is a synthetic diamond.

4. A method according to claim 3, wherein the synthetic diamond member is produced by chemical vapour deposition technology.

5. A method according to any of the preceding claims, wherein the diamond surface to be polished is heated by the relative movement of the diamond surface and the polishing surface through frictional interaction between the material of the diamond member and the material of the polishing member so that transformation of diamond to graphite is accelerated.

6. A method according to any of the preceding claims, wherein the diamond surface to be polished is heated by the relative movement of the diamond surface and the polishing surface through frictional interaction between the material of the diamond member and the material of the polishing member so that oxidation of diamond is accelerated.

7. A method according to any of the preceding claims, wherein the diamond surface to be polished is heated by the relative movement of the diamond surface and the polishing surface through frictional interaction between the material of the diamond member and the material of the polishing member so that diffusion of carbon atoms of the diamond into the polishing material takes place.

8. A method according to any of the preceding claims, wherein impact interactions between the polishing surface and the diamond surface to be polished are produced by the ultrasonic movement of the diamond surface relative to the polishing surface so that surface protrusions of the diamond surface are broken off the diamond surface.

9. A method according to any of the preceding claims, wherein the diamond surface roughness is reduced from an average roughness of approximately 5µ to approximately 0.2µ in less than two minutes.

10. A method according to any of the preceding claims, wherein the movement of the diamond surface to be polished in relation to the polishing surface is a three-dimensional movement.

11. A method according to any of the preceding claims, wherein the movement of the diamond surface to be polished in relation to the polishing surface is a two-dimensional movement wherein the plane defined by the velocity components of the movement is substantially vertical to the diamond surface.

12. A method according to any of the preceding claims, wherein the movement of the diamond surface to be polished in relation to the polishing surface is a one-dimensional movement substantially tangential to the diamond surface.

13. A method according to any of the preceding claims, wherein the ultrasonic vibrations are generated by standing or travelling waves.

14. A method according to any of the preceding claims, wherein the diamond surface to be polished and the polishing surface is moved relative to each other to increase the polished surface flatness uniformity.

15. A method according to any of the preceding claims, comprising the steps of:
producing impact interactions between the polishing surface and the diamond surface to be polished by ultrasonic movement of the diamond surface relative to the polishing surface so that surface protrusions of the diamond surface are broken off the diamond surface, and
polishing of the diamond surface with a hard material containing oxygen.

16. A method according to claim 15, further comprising the step of: polishing the diamond surface with a material in which carbon is soluble.

17. A method according to any of the preceding claims, further comprising at least one step of adding at least one active chemical between the diamond surface to be polished and the polishing surface.

18. A method according to any of the preceding claims, further comprising the step of dispensing one or more liquid(s) containing oxygen between the polishing surfaces utilizing vibration induced cavitation to increase the polishing rate.

19. A polishing apparatus for polishing a surface of a diamond member, said apparatus comprising a frame, means for mounting a diamond polishing member on the frame, means for mounting a diamond member on the frame, means for moving a polishing surface defined on the polishing member into contact with a surface of the diamond member to be polished, and ultrasonic transducer means for moving the diamond and polishing surfaces in relation to each other so as to polish the diamond surface.

20. A polishing apparatus according to claim 19, wherein the ultrasonic transducer means comprise at least two ultrasonic transducers.

21. A polishing apparatus according to claim 20, wherein the ultrasonic transducers are linear ultrasonic transducers positioned in such a way that the axes of longitudinal vibrations of the transducers are positioned substantially perpendicular to each other.

22. A polishing apparatus according to claim 20 or 21, wherein the at least two transducers are operated in different modes of vibration.
